

Patented Jan. 17, 1928.

1,656,764

## UNITED STATES PATENT OFFICE.

WILLOUGHBY STATHAM SMITH, OF NEWTON POPPLEFORD, AND HENRY JOSEPH GARNETT, OF SEVEN OAKS, ENGLAND.

### ALLOY SUITABLE FOR LOADING TELEPHONE AND TELEGRAPH CONDUCTORS.

No Drawing. Application filed April 29, 1926, Serial No. 105,564, and in Great Britain July 10, 1925.

This invention relates to new alloys which have a very high specific resistance and high initial magnetic permeability, and are consequently very suitable in the form of 5 wires, tapes or strips, for loading telephone and telegraph conductors.

According to this invention an alloy is composed of nickel 62-69%, iron 11-19%, copper 6-10%, chromium 5-9%, preferably 10 with an addition of about 0.5% manganese.

A specially suitable alloy contains nickel 65%, iron 18%, copper 10%, chromium 7% and manganese 0.5%. This alloy has an initial permeability of 1200 and electrical re- 15 sistance of 99 microhms per cm<sup>2</sup>.

What we claim is:—

1. An alloy suitable for loading telephone and telegraph conductors and having a nickel content of from 62 to 69%, an iron 20 content of from 11 to 19%, a copper content

of from 6 to 10% and a chromium content of from 5 to 9%.

2. An alloy suitable for loading telephone and telegraph conductors and having a nickel content of from 62 to 69%, an iron 25 content of from 11 to 19%, a copper content of from 6 to 10% and a chromium content of from 5 to 9%, together with an addition of about 0.5% manganese.

3. An alloy suitable for loading telephone 30 and telegraph conductors and composed of nickel 65%, iron 18%, copper 10%, chromium 7% and an addition of 0.5% of manganese.

In testimony that we claim the foregoing 35 as our invention, we have signed our names this fifteenth day of April, 1926.

WILLOUGHBY STATHAM SMITH.  
HENRY JOSEPH GARNETT.